



US012129601B2

(12) **United States Patent**  
**Vogt et al.**

(10) **Patent No.:** **US 12,129,601 B2**  
(45) **Date of Patent:** **\*Oct. 29, 2024**

(54) **MULTI-PLY TISSUE PRODUCT**

(71) Applicant: **Kimberly-Clark Worldwide, Inc.,**  
Neenah, WI (US)

(72) Inventors: **Kevin Joseph Vogt**, Neenah, WI (US);  
**Mark William Sachs**, Appleton, WI  
(US); **Christopher Steven LeCount**,  
Greenville, WI (US); **Erin Ann**  
McCormick, Neenah, WI (US); **Devon**  
**Gaynelle Curley**, Menasha, WI (US);  
**Sara Jane Wille Stabelfeldt**, Appleton,  
WI (US); **Nathan John Vogel**, Neenah,  
WI (US)

(73) Assignee: **Kimberly-Clark Worldwide, Inc.,**  
Neenah, WI (US)

(\*) Notice: Subject to any disclaimer, the term of this  
patent is extended or adjusted under 35  
U.S.C. 154(b) by 0 days.

This patent is subject to a terminal dis-  
claimer.

(21) Appl. No.: **18/369,896**

(22) Filed: **Sep. 19, 2023**

(65) **Prior Publication Data**

US 2024/0003093 A1 Jan. 4, 2024

**Related U.S. Application Data**

(63) Continuation of application No. 17/615,669, filed as  
application No. PCT/US2020/034546 on May 26,  
2020, now Pat. No. 11,795,626.  
(60) Provisional application No. 62/856,411, filed on Jun.  
3, 2019.

(51) **Int. Cl.**

**D21H 27/40** (2006.01)  
**D21H 27/00** (2006.01)  
**D21H 27/02** (2006.01)

(52) **U.S. Cl.**

CPC ..... **D21H 27/40** (2013.01); **D21H 27/007**  
(2013.01); **D21H 27/02** (2013.01)

(58) **Field of Classification Search**

CPC ..... D21H 27/40; D21H 27/007; D21H 27/02;  
D21H 21/146; D21H 27/30; D21H  
27/002; B31F 1/14; B31F 1/126

See application file for complete search history.

(56) **References Cited**

U.S. PATENT DOCUMENTS

4,886,579 A 12/1989 Clark et al.  
9,121,137 B2 9/2015 Mazmensky et al.

|                   |         |                          |
|-------------------|---------|--------------------------|
| 9,951,477 B2      | 4/2018  | Zwick et al.             |
| 10,132,041 B2     | 11/2018 | Hermans et al.           |
| 10,145,069 B2     | 12/2018 | Shannon et al.           |
| 10,337,148 B2     | 7/2019  | Rouse et al.             |
| 10,337,149 B2     | 7/2019  | Rouse et al.             |
| 10,385,516 B2     | 8/2019  | Zawadzki et al.          |
| 10,428,465 B2     | 10/2019 | Rouse et al.             |
| 10,487,452 B1     | 11/2019 | Qin et al.               |
| 10,550,522 B2     | 2/2020  | Shannon et al.           |
| 10,947,673 B2     | 3/2021  | Rouse et al.             |
| 11,053,643 B2     | 7/2021  | Rouse et al.             |
| 11,427,968 B2 *   | 8/2022  | Vogt ..... A47K 10/16    |
| 11,795,626 B2 *   | 10/2023 | Vogt ..... B31F 1/126    |
| 2004/0084165 A1   | 5/2004  | Shannon et al.           |
| 2006/0130986 A1   | 6/2006  | Flugge-Berendes et al.   |
| 2007/0144697 A1   | 6/2007  | Dyer et al.              |
| 2008/0073045 A1   | 3/2008  | Dyer et al.              |
| 2014/0178660 A1   | 6/2014  | Kim et al.               |
| 2015/0240426 A1   | 8/2015  | Hermans et al.           |
| 2016/0097163 A1   | 4/2016  | Rekoske et al.           |
| 2016/0145809 A1   | 5/2016  | Hermans et al.           |
| 2018/0142419 A1   | 5/2018  | Rouse et al.             |
| 2018/0142421 A1   | 5/2018  | Rouse et al.             |
| 2020/0035456 A1   | 1/2020  | Fan et al.               |
| 2020/0102705 A1   | 4/2020  | Rouse et al.             |
| 2020/0115853 A1   | 4/2020  | Shannon et al.           |
| 2021/0156093 A1   | 5/2021  | Rouse et al.             |
| 2021/0238806 A1   | 8/2021  | Tirimacco                |
| 2021/0277603 A1   | 9/2021  | Anderson et al.          |
| 2021/0285159 A1   | 9/2021  | Burazin et al.           |
| 2021/0292973 A1   | 9/2021  | Rouse et al.             |
| 2022/0090324 A1 * | 3/2022  | Vogt ..... D21H 27/40    |
| 2022/0364310 A1 * | 11/2022 | Vogt ..... D21H 27/005   |
| 2023/0072598 A1 * | 3/2023  | Lindsay ..... D21H 27/40 |
| 2023/0143624 A1 * | 5/2023  | Satori ..... D21H 27/002 |
|                   |         | 162/123                  |
| 2023/0148320 A1 * | 5/2023  | Satori ..... D21H 27/02  |
|                   |         | 162/111                  |
| 2024/0003093 A1 * | 1/2024  | Vogt ..... D21H 21/146   |

**FOREIGN PATENT DOCUMENTS**

|    |               |         |
|----|---------------|---------|
| WO | 2020205520 A1 | 10/2020 |
| WO | 2020205524 A1 | 10/2020 |
| WO | 2020247205 A1 | 12/2020 |

\* cited by examiner

*Primary Examiner* — Jose A Fortuna

(74) *Attorney, Agent, or Firm* — KIMBERLY-CLARK  
WORLDWIDE, INC.

(57) **ABSTRACT**

Disclosed are non-treated, creped tissue webs, and tissue products produced therefrom, having low stiffness and surface lint. The inventive products may be produced by a print creping process adapted to dispose a non-crosslinked latex polymer on at least one of the outer surfaces of the tissue product. The non-crosslinked latex polymer creping composition does not negatively affect stiffness such that the products generally have a Stiffness Index less than about 5.0, such as from about 2.5 to about 5.0.

**19 Claims, 5 Drawing Sheets**



FIG. 1



FIG. 2



FIG. 3



FIG. 4



FIG. 5



FIG. 6



FIG. 7

## MULTI-PLY TISSUE PRODUCT

## BACKGROUND

Absorbent paper products such as paper towels, facial tissues and other similar products are designed to include several important properties. For example, the products should have good bulk, a soft feel and should be highly absorbent. The product should also have good strength even while wet and should resist tearing. Unfortunately, it is very difficult to produce a high strength paper product that is also soft and highly absorbent. Usually, when steps are taken to increase one property of the product, other characteristics of the product are adversely affected. For instance, softness is typically increased by decreasing or reducing fiber bonding within the paper product. Inhibiting or reducing fiber bonding, however, adversely affects the strength of the paper web.

One tissue manufacturing process for balancing often competing physical properties is disclosed in U.S. Pat. No. 7,462,258. The process may be adapted to print binder on one or both sides of a fibrous web and typically involves a single creping step after the binder is applied. The binder is a crosslinked latex and comprises an azetidinium-reactive polymer. The presence of an azetidinium-reactive polymer enables the binder to crosslink both with itself and cellulose of the fibrous web. In this manner, the crosslinked latex of the '258 patent forms covalent bonds with cellulose of the fibrous web. Thus, while the '258 discloses a process for producing tissue products having good bulk, softness and absorbency, the binder is covalently bonded to the cellulose of the fibrous web and impedes the web from dispersing when wetted.

Alternatives to the crosslinked latex binders of the '258 patent are disclosed in U.S. Pat. No. 9,121,137, which discloses a crosslinked latex binder comprising a primary polymer and a polyfunctional aldehyde. The polyfunctional aldehyde, like the azetidinium-reactive polymer contained in the binders of the '258 patent, enables the binder to form covalent bonds with cellulose. As such, products produced according to the '137 patent retain a significant portion of their tensile strength after being wetted, even after an extended period of time.

Accordingly, there remains a need in the art for a tissue manufacturing process for balancing the often competing physical properties, such as bulk, hand-feel and absorbency, while also providing a product that is readily dispersible.

## SUMMARY

The present invention provides creped tissue webs, and multi-ply tissue products produced therefrom. Generally, the products have improved properties, such as low stiffness and surface lint, even though they do not have a surface treatment such as silicones, waxes, lotions or quaternary ammonium compounds comprising alkyl chains.

The inventive products generally comprise two or more tissue plies, such as two, three or four plies. At least one of the plies, and preferably two or more of the plies, have been prepared by a creping process and more preferably by a print crepe process. In certain preferred embodiments, one or more of the plies are prepared by a print crepe process that disposes a non-crosslinked latex polymer on an outer surface of the ply. Without being bound by any particular theory, it is believed that the presence of a non-crosslinked latex polymer improves certain surface properties, such as smoothness, and may also improve durability. Surprisingly,

however, the non-crosslinked latex polymer does not negatively affect stiffness (measured as Stiffness Index) such that products produced according to the present invention generally have a Stiffness Index less than about 5.0, such as from about 2.5 to about 5.0.

In other embodiments, multi-ply tissue products of the present invention have low levels of surface lint, which may be measured as Slough. Surface lint generally results from the release of loosely bound fibers from the surface of the tissue product in use and is often an issue when producing soft, low stiffness tissue products. Despite this trend, the inventive tissue products surprisingly have both low Slough, such as a Slough less than about 5.0 mg, and a low degree of stiffness, such as Stiffness Index less than about 5.0. For example, in one embodiment the present invention provides a tissue product comprising a spirally wound non-treated creped multi-ply tissue product having a geometric mean tensile (GMT) of about 1,000 g/3" or greater, a Stiffness Index less than about 5.0 and a Slough less than about 5.0 mg.

In yet other embodiment the invention provides a non-treated and creped tissue product having good strength and durability. For example, the invention provides a non-treated and creped multi-ply tissue product comprising a first non-treated and creped tissue ply and a second non-treated and creped tissue ply, the non-treated and creped multi-ply tissue product having a geometric mean tensile (GMT) of about 1,000 g/3" or greater and a geometric mean tensile energy absorption (GM TEA) greater than about 20 gf·cm/cm<sup>2</sup>.

In still other embodiments the present invention provides rolled tissue products, particularly rolled products comprising a multi-ply tissue product spirally wound about the core. In certain instances the multi-ply tissue product may comprise at least one non-treated and creped tissue ply having a first outer surface comprising a plurality of embossments and a non-crosslinked latex polymer disposed thereon, the multi-ply tissue product having a basis weight from about 48.0 to about 60.0 gsm, a GMT of about 1,000 g/3" or greater and a Slough less than about 5.0 mg.

In still other embodiments the present invention provides tissue products well suited for use as bath tissue. For example, the invention provides tissue products having a Slosch time less than about 2 minutes. In particularly preferred embodiments the invention provides a non-treated and creped multi-ply tissue product comprising a first non-treated and creped tissue ply, a second non-treated and creped tissue ply, a creping composition consisting essentially of a non-crosslinked vinyl acetate-ethylene polymer and optionally an anti-blocking agent disposed on the first and the second tissue ply and a plurality of embossments disposed on the first or the second tissue ply, wherein the product has a GMT from about 1,000 to about 2,500 g/3" and a Slosch time less than about 2 minutes.

## DESCRIPTION OF THE DRAWINGS

FIG. 1 illustrates one embodiment for forming a multi-layered tissue web according to the present invention;

FIG. 2 illustrates one embodiment for forming a basesheet useful in the production of a tissue product according to the present invention;

FIG. 3 illustrates one embodiment of a print-crepe process for producing a tissue product according to the present invention;

FIG. 4 illustrates one pattern for applying a binder to a basesheet;

## 3

FIG. 5 illustrates another pattern for applying a binder to a basesheet;

FIG. 6 illustrates still another pattern for applying a binder to a basesheet; and

FIG. 7 illustrates a test specimen prepared for Slough testing.

## DEFINITIONS

As used herein the term "Basesheet" refers to a tissue web formed by any one of the papermaking processes described herein that has not been subjected to further processing, such as embossing, calendering, treatment with a binder or softening composition, perforating, plying, folding, or rolling into individual rolled products.

As used herein the term "Tissue Product" refers to products made from basesheets and includes, bath tissues, facial tissues, paper towels, industrial wipers, foodservice wipers, napkins, medical pads, and other similar products.

As used herein the term "Ply" refers to a discrete tissue web used to form a tissue product. Individual plies may be arranged in juxtaposition to each other.

As used herein, the term "Layer" refers to a plurality of strata of fibers, chemical treatments, or the like, within a ply. The term "Layered Tissue Web" generally refers to a tissue web formed from two or more layers of aqueous papermaking furnish. In certain instances, the aqueous papermaking furnish forming two or more of the layers comprise different fiber types.

As used herein the term "Basis Weight" generally refers to the conditioned weight per unit area of a tissue and is generally expressed as grams per square meter (gsm). Basis weight is measured as described in the Test Methods section below. While the basis weights of tissue products prepared according to the present invention may vary, in certain embodiments the products have a basis weight greater than about 20 gsm, such as greater than about 30 gsm, such as greater than about 40 gsm, such as from about 20 to about 80 gsm, such as from about 30 to about 60 gsm, such as from about 45 to about 55 gsm.

As used herein, the term "Caliper" refers to the thickness of a tissue product, web, sheet or ply, typically having units of microns ( $\mu\text{m}$ ) and is measured as described in the Test Methods section below.

As used herein, the term "Bulk" refers to the quotient of the caliper ( $\mu\text{m}$ ) of a product or ply divided by the bone dry basis weight (gsm). The resulting bulk is expressed in cubic centimeters per gram (cc/g). Tissue products prepared according to the present invention may, in certain embodiments, have a bulk greater than about 8.0 cc/g, more preferably greater than about 9.0 cc/g and still more preferably greater than about 10.0 cc/g, such as from about 8.0 to about 12.0 cc/g.

As used herein, the term "Slope" refers to the slope of the line resulting from plotting tensile versus stretch and is an output of the MTS TestWorks™ in the course of determining the tensile strength as described in the Test Methods section herein. Slope is reported in the units of grams (g) per unit of sample width (inches) and is measured as the gradient of the least-squares line fitted to the load-corrected strain points falling between a specimen-generated force of 70 to 157 grams (0.687 to 1.540 N) divided by the specimen width.

As used herein, the term "Geometric Mean Slope" (GM Slope) generally refers to the square root of the product of machine direction slope and cross-machine direction slope. While the GM Slope may vary amongst tissue products prepared according to the present disclosure, in certain

## 4

embodiments, tissue products may have a GM Slope less than about 10.00 kg, more preferably less than about 9.00 kg and still more preferably less than about 8.00 kg, such as from about 6.00 to about 10.0 kg, such as from about 6.00 to about 8.00 kg.

As used herein, the term "Geometric Mean Tensile" (GMT) refers to the square root of the product of the machine direction tensile strength and the cross-machine direction tensile strength of the web.

As used herein, the term "Stiffness Index" refers to the quotient of the geometric mean tensile slope, defined as the square root of the product of the MD and CD slopes (having units of kg), divided by the geometric mean tensile strength (having units of grams per three inches).

Stiffness Index =

$$\frac{\sqrt{MD \text{ Tensile Slope (kg)} \times CD \text{ Tensile Slope (kg)}}}{GMT(\text{g/3''})} \times 1,000$$

While the Stiffness Index of tissue products prepared according to the present disclosure may vary, in certain instances the Stiffness Index ranges from about 2.5 to about 5.0, such as from about 3.0 to about 4.5, such as from about 3.0 to about 4.0.

As used herein, the term "TEA Index" refers to the geometric mean tensile energy absorption (having units of  $\text{g}\cdot\text{cm}/\text{cm}^2$ ) at a given geometric mean tensile strength (having units of grams per three inches) as defined by the equation:

$$TEA \text{ Index} = \frac{GM \text{ TEA}(\text{g}\cdot\text{cm}/\text{cm}^2)}{GMT(\text{g/3''})} \times 100$$

While the TEA Index may vary, in certain instances tissue products prepared according to the present disclosure have a TEA Index greater than about 1.50, such as greater than about 1.75, such as greater than about 2.00, such as from about 1.50 to about 2.25, such as from about 1.75 to about 2.25.

As used herein, the term "Slough" generally refers to the undesirable sloughing off of bits of the tissue web when rubbed and is generally measured as described in the Test Methods section below. Slough is generally reported in terms of mass, such as milligrams (mg). While the Slough of inventive tissue products may vary, in certain instances tissue products prepared according to the present invention have a Slough less than about 5.0 mg and more preferably less than about 3.0 mg, such as from about 0.20 to about 5.0, such as from about 0.50 to about 3.0 mg.

As used herein, the term "TS750" generally refers to the smoothness of a tissue product surface measured using an EMTEC Tissue Softness Analyzer ("Emtec TSA") (Emtec Electronic GmbH, Leipzig, Germany) interfaced with a computer running Emtec TSA software (version 3.19 or equivalent). The units of the TS750 value are dB V<sup>2</sup>rms, however, TS750 values are often referred to herein without reference to units. Generally, the TS750 value is the magnitude of the peak occurring at a frequency between about 200 and 1,000 Hz, which is produced by vibration of the tissue membrane during the test procedure. Generally, a lower TS750 value is indicative of a smoother surface.

As used herein, the term "Slosh" generally refers to the time needed to break-up a tissue sample into pieces less than

25×25 mm using the Slosh test as described in U.S. Pat. No. 8,257,553, the contents of which are hereby incorporated by reference in a manner consistent with the present disclosure. Generally, Slosh has units of seconds or minutes. The Slosh test uses a bench-scaled apparatus to evaluate the breakup or dispersibility of flushable consumer products as they travel through the wastewater collection system.

As used herein, the term “Wet/Dry Ratio” refers to the ratio of the wet cross-machine direction (CD) tensile strength to the dry CD tensile strength. Wet and dry CD tensile are measured as set forth in the Test Methods section below. The Wet/Dry Ratio of inventive tissue products may vary depending on several factors such as, for example, the creping composition and the amount of wet strength additive, however, in certain instances the inventive tissue products may have a Wet/Dry Ratio greater than about 0.100, such as greater than about 0.125, such as greater than about 0.150, from about 0.100 to about 0.200, such as from about 0.100 to about 0.175.

As used herein the term “permanent wet strength agent” generally refers to a chemical composition which allows a tissue product, when placed in an aqueous medium, to keep a majority of its initial tensile strength for a period of time greater than at least about 2 minutes. Permanent wet strength resins include, for example, diethylenetriamine (DETA), triethylenetetramine (TETA), tetraethylenepentamine (TEPA), epichlorhydrin resin(s), and polyamide-epichlorohydrin (PAE).

As used herein the term “non-treated” generally refers to a product, or plies of a product, that has not been treated with a papermaking additive after it has been substantially dried, such as by pressing the product against a heated rotary dryer and creping it therefrom. In particular instances non-treated product tissue products according to the present invention have not been treated by coating, spraying, rotogravure printing, flexographic printing, or extruding a wax, such as paraffin and beeswax, an oil, such as mineral oil or silicone oil, and more complex lubricants and emollients such as quaternary ammonium compounds with long alkyl chains, functional silicones, fatty acids, fatty alcohols and fatty esters, onto the surface of the product or plies after it has been substantially dried.

#### DETAILED DESCRIPTION

In general, the present disclosure is directed to creped tissue webs, and products produced therefrom. The creped webs and products generally have one or more desirable properties, such as good strength, flexibility (measured as Stiffness Index), low amounts of surface lint (measured as Slough) and a smooth surface (measured as TS750). One or more of the foregoing properties may be achieved by creping, but without the treatment with surface additives commonly used in the art such as, for example, waxes, oils and emollients such as quaternary ammonium compounds with long alkyl chains, functional silicones, fatty acids, fatty alcohols and fatty esters. In this manner, in certain preferred embodiments, the only additive present on the outer surface of the tissue product is a creping composition, which in certain preferred embodiments comprises a non-cross linked latex polymer.

In addition to being non-treated, it is generally preferred that the tissue products are void of permanent wet strength agents, such as diethylenetriamine (DETA), triethylenetetramine (TETA), tetraethylenepentamine (TEPA), epichlorhydrin resin(s), and polyamide-epichlorohydrin (PAE). The absence of a permanent wet strength ensures that the prod-

ucts readily disperse in an aqueous environment. As such, the products of the present invention are readily dispersible in water and well suited for use as bath tissue. In certain embodiments the products of the present invention may have a Slosh time less than 2 minutes, such as less than about 110 seconds, such as less than about 60 seconds, such as less than about 30 seconds, such as from about 10 seconds to 2 minutes, such as from about 10 seconds to about 60 seconds, such as from about 15 seconds to about 45 seconds.

Another desirable property of the inventive tissue products is a high degree of flexibility, such as a Stiffness Index less than about 5.0, such as less than about 4.5, such as less than about 4.0. In certain instances, the inventive products may have a Stiffness Index from about 2.5 to about 5.0, such as from about 3.0 to about 4.5, such as from about 3.0 to about 4.0. The foregoing Stiffness Index may be achieved at geometric tensile (GMT) strengths of about 1,000 g/3" or greater, such as about 1,250 g/3" or greater, such as 1,500 g/3" or greater, such as from about 1,000 to about 2,500 g/3", such as from about 1,000 to about 2,200 g/3", such as from about 1,500 to about 2,000 g/3".

In other embodiments the inventive tissue products have relatively low geometric mean slopes (GM Slope), such as less than about 10.0 kg, such as less than about 8.0 kg, such as less than about 6.0, such as from about 4.0 to about 10.0 kg, such as from about 5.0 to about 8.0 kg. At the foregoing GM Slopes, the products may have a Stiffness Index from about 2.5 to about 5.0, such as from about 3.0 to about 4.5, such as from about 3.0 to about 4.0. In certain instances the foregoing Stiffness Index may be achieved at geometric tensile strengths greater than about 1,200 g/3", such as greater than about 1,400 g/3", such as greater than about 1,600 g/3", such as from about 1,200 to about 3,000 g/3", such as from about 1,500 to about 2,500 g/3", such as from about 1,750 to about 2,500 g/3", such as from about 1,750 to about 2,000 g/3".

In still other embodiments, tissue products of the present invention have improved surface smoothness, even in those instances where they are non-treated and embossed. For example, the non-treated tissue products may have an embossing pattern that provides the product with aesthetic appeal and good bulk but still maintains a relatively smooth surface, such as a TS750 value less than about 40.0, such as less than about 30.0, such as less than about 25.0, such as from about 15.0 to 40.0, such as from about 20.0 to about 35.0. Generally, a lower TS750 value indicates a smoother surface. In other instances, the tissue products may have a bulk greater than about 10.0 cc/g and a TS750 value less than about 40.0.

In yet other embodiments the present invention provides a non-treated multi-ply tissue product having improved surface smoothness and low degrees of stiffness. For example, the inventive products may have a Stiffness Index from about 2.5 to about 5.0, such as from about 3.0 to about 4.5, such as from about 3.0 to about 4.0 and a TS750 value less than 40.0 and more preferably less than about 30.0 and still more preferably less than about 25.0, such as from about 15.0 to 40.0, such as from about 20.0 to about 35.0.

In particularly preferred embodiments the tissue products comprise two or more creped tissue plies, wherein at least one of the plies is embossed and the product has a TS750 from about 15.0 to 40.0 and a Stiffness Index from about 2.5 to about 5.0. The foregoing TS750 values may be archived at relatively high degrees of strength and substance, such as a GMT from about 1,000 to about 2,500 g/3" and a basis weight from about 48.0 to about 58.0 gsm.

Another desirable property of the inventive tissue products is relatively low degrees of surface lint, such as a Slough less than about 5.0 mg and more preferably less than about 3.0 mg, such as from about 0.20 to about 5.0, such as from about 0.50 to about 3.0 mg. Surprisingly, the foregoing Slough levels may be achieved even in those instances where the product is creped and has a relatively high basis weight, such as a basis weight of about 45 grams per square meter (gsm) or greater, such as about 48 gsm or greater, such as about 50 gsm or greater, such as from about 45 to about 60 gsm, such as from about 48 to about 58 gsm. Typically, increased basis weight, and the often-associated higher caliper, result in increased surface lint, particularly when the product is creped. Despite this trend, the present invention surprisingly provides a high basis weight tissue product having low degrees of surface lint, such as a product having a basis weight from about 48 to about 58 gsm and a Slough from about 0.50 to about 3.0 mg.

Although the products are generally smooth and flexible, they are highly durable. For example, in certain instances the non-treated products of the present invention may have a geometric mean tensile energy absorption (GM TEA) greater than about 20 grams force-centimeters per square centimeter ( $gf\cdot cm/cm^2$ ), more preferably greater than about 22  $gf\cdot cm/cm^2$ , still more preferably greater than about 24  $g\cdot cm/cm^2$ , such as from about 20 to about 45  $gf\cdot cm/cm^2$ , such as from about 25 to about 45  $gf\cdot cm/cm^2$ , such as from about 30 to about 40  $gf\cdot cm/cm^2$ .

In yet other embodiments the inventive tissue products have a GM TEA greater than about 20  $gf\cdot cm/cm^2$ , such as from about 20 to about 45  $gf\cdot cm/cm^2$ , and a dry burst strength greater than about 700 gf, such as from about 700 to about 1,000 gf, such as from about 800 to about 1,000 gf.

In certain instances the tissue products have a high degree of durability, even at modest levels of tensile strength such that the products have a TEA Index greater than about 1.50, such from about 1.50 to about 1.75. A comparison of the physical properties, including GM TEA and Stiffness Index, of inventive and several commercially available tissue products may be found in Table 1, below.

TABLE 1

|                                            | Through-air<br>Dried | Creped | GMT<br>( $g/3"$ ) | GM<br>TEA<br>( $gf\cdot cm/cm^2$ ) | GM<br>Slope<br>(kg) | Stiffness<br>Index |
|--------------------------------------------|----------------------|--------|-------------------|------------------------------------|---------------------|--------------------|
| Angel Soft                                 | N                    | Y      | 758               | 10.90                              | 7.87                | 10.39              |
| Charmin<br>Sensitive                       | Y                    | Y      | 761               | 11.17                              | 8.75                | 11.50              |
| Charmin Ultra<br>Soft                      | Y                    | Y      | 715               | 11.74                              | 4.96                | 6.94               |
| Charmin Ultra<br>Strong                    | Y                    | Y      | 1102              | 13.27                              | 7.84                | 7.12               |
| Cottonelle Ultra<br>Comfort Care           | Y                    | N      | 990               | 11.25                              | 6.43                | 6.50               |
| Great Value<br>Ultra Soft                  | Y                    | Y      | 1050              | 8.12                               | 10.70               | 10.19              |
| Great Value<br>Ultra Strong                | Y                    | Y      | 1347              | 11.73                              | 8.67                | 6.43               |
| Quilted<br>Northern Ultra<br>Plush         | N                    | Y      | 665               | 11.36                              | 4.94                | 7.43               |
| Quilted<br>Northern Ultra<br>Soft & Strong | N                    | Y      | 1286              | 11.44                              | 5.86                | 4.56               |
| Target UP &<br>Up Soft                     | Y                    | Y      | 802               | 9.93                               | 7.63                | 9.52               |
| Target Up &<br>Up Ultra Soft               | Y                    | Y      | 1101              | 9.63                               | 9.83                | 8.93               |

TABLE 1-continued

|                                       | Through-air<br>Dried | Creped | GMT<br>( $g/3"$ ) | GM<br>TEA<br>( $gf\cdot cm/cm^2$ ) | GM<br>Slope<br>(kg) | Stiffness<br>Index |
|---------------------------------------|----------------------|--------|-------------------|------------------------------------|---------------------|--------------------|
| White Cloud<br>Ultra Bath<br>Tissue   | Y                    | Y      | 1212              | 14.50                              | 10.67               | 8.80               |
| White Cloud<br>Ultra Soft &<br>Strong | Y                    | Y      | 1278              | 14.59                              | 9.66                | 7.56               |
| Inventive 1                           | Y                    | Y      | 1977              | 30.2                               | 10.00               | 5.06               |
| Inventive 2                           | Y                    | Y      | 1365              | 23.1                               | 5.70                | 4.17               |

15 In other embodiments the inventive non-treated, multi-ply creped tissue products have a relatively high degree of stretch, such as a geometric mean stretch (GM Stretch) greater than about 20 percent, more preferably greater than about 22 percent and still more preferably greater than about 24 percent, such as from about 20 to about 30 percent, such as from about 22 to about 28 percent. The combination of 20 relatively high stretch and good durability, such as a GM Stretch from about 22 to about 28 percent and a GM TEA greater than about 20  $gf\cdot cm/cm^2$ , provides the tissue products with improved poke-through resistance, which is particularly important for bath tissue, but can be equally beneficial for facial tissue and towels.

25 In yet other embodiments the present invention provides a non-treated, multi-ply creped tissue product that retains a relatively high degree of strength when wet. For example, 30 the invention provides products devoid of permanent wet strength agents and having a Wet/Dry Ratio greater than about 0.100, such as greater than about 0.125, such as greater than about 0.150, such as from about 0.100 to about 0.200, such as from about 0.100 to about 0.150. In certain 35 instances, the tissue products may have a wet CD tensile strength greater than about 100  $g/3"$ , and more preferably greater than about 120  $g/3"$ , and more preferably greater than about 140  $g/3"$ , such as from about 120 to about 200  $g/3"$ , and a Wet/Dry Ratio greater than about 0.100. The 40 foregoing wet tensile properties are generally achieved without the use of a permanent wet strength agent and without topically treating the tissue with surface additives such as polysiloxanes, waxes or lotions.

45 In certain embodiments tissue products may be formed from one or more basesheets, which may comprise a single homogenous or blended layer, or be multi-layered. In those instances where the basesheet is multi-layered it may comprise, two, three, or more layers. For example, the basesheet 50 may comprise three layers such as first and second outer layers and a middle layer disposed there between. The layers may comprise the same or different fiber types. For example, the first and second outer layers may comprise short, low coarseness wood pulp fibers, such as hardwood kraft pulp fibers, and the middle layer may comprise long, low coarseness wood pulp fibers, such as northern softwood kraft pulp 55 fibers.

60 In those instances where the web comprises multiple layers, the relative weight percentage of each layer may vary. For example, the web may comprise first and second outer layers and a middle layer where the first outer layer comprises from about 25 to about 35 weight percent of the layered web, the middle layer comprises from about 30 to about 50 weight percent of the layered web and the second outer layer comprises from about 25 to about 35 weight percent of the layered web.

65 Multi-layered basesheets useful in the present invention may be formed using any number of different processes

known in the art, such as the process disclosed in U.S. Pat. No. 5,129,988, the contents of which are incorporated herein in a manner consistent with the present disclosure. One process for a forming multi-layered basesheet is illustrated in FIG. 1. A dilute aqueous suspension of papermaking fibers is dispersed from a headbox 10 having an upper headbox wall 12 and a lower headbox wall 14 and first and second dividers 16, 18. In this manner the headbox may be used to form a basesheet having outer layers 22, 24 and a middle layer 20, where each of the layers may comprise the same or different papermaking fibers.

To form the multi-layered basesheet, an endless traveling forming fabric 26, suitably supported and driven by rolls 28 and 30, receives the layered papermaking stock issuing from headbox 10. Once retained on fabric 26, the layered fiber suspension passes water through the fabric as shown by the arrows 32. Water removal is achieved by combinations of gravity, centrifugal force and vacuum suction depending on the forming configuration.

In certain embodiments the one or more layers of a multi-layered basesheet, such as the middle layer, may be formed without a substantial amount of inner fiber-to-fiber bond strength. In this regard, the fiber furnish used to form a given layer can be treated with a chemical debonding agent. The debonding agent can be added to the fiber slurry during the pulping process or can be added directly to the fiber slurry prior to the headbox. Suitable debonding agents that may be used in the present invention include cationic debonding agents, particularly quaternary ammonium compounds, mixtures of quaternary ammonium compounds with polyhydroxy compounds, and modified polysiloxanes.

Suitable cationic debonding agents include, for example, fatty dialkyl quaternary amine salts, mono fatty alkyl tertiary amine salts, primary amine salts, imidazoline quaternary salts and unsaturated fatty alkyl amine salts. Other suitable debonding agents are disclosed in U.S. Pat. No. 5,529,665, the contents of which are incorporated herein in a manner consistent with the present disclosure. In one embodiment, the debonding agent used in the process of the present invention is an organic quaternary ammonium chloride, such as those available under the trademark ProSoft™ (Solenis, Wilmington, DE). The debonding agent can be added to the fiber slurry in an amount of from about 1.0 kg per metric ton to about 15 kg per metric ton of fibers present within the slurry.

Particularly useful quaternary ammonium debonders include imidazoline quaternary ammonium debonders, such as oleyl-imidazoline quaternaries, dialkyl dimethyl quaternary debonders, ester quaternary debonders, diamidoamine quaternary debonders, and the like. The imidazoline-based debonding agent can be added in an amount of between 1.0 to about 10 kg per metric ton.

In other embodiments, a layer or other portion of the basesheet, including the entire basesheet, may optionally include a temporary wet strength agent. As used herein "temporary wet strength agents" are those which show less than 50 percent of their original wet strength after being saturated with water for five minutes. Suitable temporary wet strength agents include materials that can react with hydroxyl groups, such as on cellulosic pulp fibers, to form hemiacetal bonds that are reversible in the presence of excess water. Suitable temporary wet strength agents are known to those of ordinary skill in the art. Non-limiting examples of temporary wet strength agents suitable for the fibrous structures of the present invention include glyoxalated polyacrylamide polymers, for example cationic glyoxalated polyacrylamide polymers. Temporary wet strength

agents useful in the present invention may have average molecular weights of from about 20,000 to about 400,000, such as from about 50,000 to about 400,000, such as from about 70,000 to about 300,000, such as about 100,000 to about 200,000. In certain instances the temporary wet strength agent may comprise a commercially available temporary wet strength agent such as those marketed under the trademark Herco-bond™ (Solenis, Wilmington, DE) or Fennobond™ (Kemira Chemicals, Inc., Atlanta, GA).

In other instances the basesheet may optionally include a dry strength additive, such as carboxymethyl cellulose resins, starch based resins, and mixtures thereof. Particularly preferred dry strength additives are cationic starches, and mixtures of cationic and anionic starches. In certain instances, the dry strength agent may comprise a commercially available modified starch such as marketed under the trademark RediBOND™ (Ingredion, Westchester, IL) or a commercially available carboxymethyl cellulose resin such as those marketed under the trademark Aqualon™ (Ashland LLC, Bridgewater, NJ). The amount of wet strength agent or dry strength added to the pulp fibers can be at least about 0.1 dry weight percent, more specifically about 0.2 dry weight percent or greater, and still more specifically from about 0.1 to about 3.0 dry weight percent, based on the dry weight of the fibers.

Tissue basesheets useful in forming tissue products of the present invention may be formed using any one of several well-known manufacturing processes. For example, in certain embodiments, tissue products may be produced by a through-air drying (TAD) manufacturing process, an advanced tissue molding system (ATMOS) manufacturing process, a structured tissue technology (STT) manufacturing process, a conventional wet pressed (also referred to as "CTEC") manufacturing process or a belt creped manufacturing process. In particularly preferred embodiments the tissue product is manufactured by a creped through-air dried (CTAD) process or uncreped through-air dried (UCTAD) process.

With reference now to FIG. 2, a method for making through-air dried paper sheets is illustrated. Shown is a twin wire former having a papermaking headbox 34, such as a layered headbox, which injects or deposits a stream 36 of an aqueous suspension of papermaking fibers onto the forming fabric 38 positioned on a forming roll 39. The forming fabric serves to support and carry the newly-formed wet web downstream in the process as the web is partially dewatered to a consistency of about 10 dry weight percent. Additional dewatering of the wet web can be carried out, such as by vacuum suction, while the wet web is supported by the forming fabric.

The wet web is then transferred from the forming fabric to a transfer fabric 40. In one embodiment, the transfer fabric can be traveling at a slower speed than the forming fabric in order to impart increased stretch into the web. This is commonly referred to as a "rush" transfer. The relative speed difference between the two fabrics can be from 0 to 60 percent, more specifically from about 15 to 45 percent. Transfer is preferably carried out with the assistance of a vacuum shoe 42 such that the forming fabric and the transfer fabric simultaneously converge and diverge at the leading edge of the vacuum slot.

The web is then transferred from the transfer fabric to the through-air drying fabric 44 with the aid of a vacuum transfer roll 46 or a vacuum transfer shoe, optionally again using a fixed gap transfer as previously described. The through-air drying fabric can be traveling at about the same

## 11

speed or a different speed relative to the transfer fabric. If desired, the through-air drying fabric can be run at a slower speed to further enhance stretch. Transfer can be carried out with vacuum assistance to ensure deformation of the sheet to conform to the through-air drying fabric, thus yielding desired bulk and imparting the web with a three-dimensional topographical pattern. Suitable through-air drying fabrics are described, for example, in U.S. Pat. Nos. 6,998,024, 7,611,607 and 10,161,084, the contents of which are incorporated herein by reference in a manner consistent with the present disclosure.

In one embodiment, the through-air drying fabric comprises a single layer fabric woven from shute and warp filaments. In certain instances the shute filaments may comprise two or more different diameters and may be interwoven with the warp filaments so as to form a textured sheet contacting surface having substantially continuous machine-direction ripples separated by valleys. In other instances the woven fabric may comprise a plurality of substantially continuous machine-direction ripples formed of multiple warp strands grouped together and supported by multiple shute strands of two or more diameters. During drying, the web can be macroscopically arranged to conform to the surface of the through-air drying fabric and form a textured, three-dimensional surface.

The side of the web contacting the through-air drying fabric is typically referred to as the "fabric side" of the paper web. The fabric side of the paper web, as described above, may have a shape that conforms to the surface of the through-air drying fabric after the fabric is dried in the through-air dryer. The opposite side of the paper web, on the other hand, is typically referred to as the "air side."

The level of vacuum used for the web transfers can be from about 3 to about 15 inches of mercury (75 to about 380 millimeters of mercury), preferably about 5 inches (125 millimeters) of mercury. The vacuum shoe (negative pressure) can be supplemented or replaced by the use of positive pressure from the opposite side of the web to blow the web onto the next fabric in addition to or as a replacement for sucking it onto the next fabric with vacuum. Also, a vacuum roll or rolls can be used to replace the vacuum shoe(s).

While supported by the through-air drying fabric, the web is dried to a consistency of about 94 percent or greater by the through-air dryer 48 and thereafter transferred to a carrier fabric 50. The dried basesheet 52 is transported to the reel 54 using carrier fabric 50 and an optional carrier fabric 56. An optional pressurized turning roll 58 can be used to facilitate transfer of the web from carrier fabric 50 to fabric 56.

In one embodiment, the reel 54 shown in FIG. 2 can run at a speed slower than the fabric 56 in a rush transfer process for building bulk into the paper web 52. For instance, the relative speed difference between the reel and the fabric can be from about 5 to about 25 percent and, particularly from about 12 to about 14 percent. Rush transfer at the reel can occur either alone or in conjunction with a rush transfer process upstream, such as between the forming fabric and the transfer fabric.

Once the web is formed, a binder composition is applied to at least one side of the web. In this manner, the present invention provides a tissue product comprising a web having first and second outer surfaces, wherein at least one outer surface comprises a topically applied binder, particularly a binder applied in a network. As used herein, the term "network" is used to describe any binder pattern that serves to bond the sheet together. The pattern can be regular or irregular and can be continuous or discontinuous.

## 12

With reference now to FIG. 3, one embodiment of applying a binder material to one outer surface of a web is illustrated. Shown is paper web 52 passing through a binder material application station 65. Station 65 includes a transfer roll 67 in contact with a rotogravure roll 68, which is in communication with a reservoir 69 containing a suitable binder 70. Although gravure printing of the binder is illustrated, other means of applying the binder material can also be used, such as foam application, spray application, flexographic printing, or digital printing methods, such as ink jet printing, and the like. The rotogravure roll 68 applies binder material 70 to one side of the web 52 in a pre-selected pattern.

FIGS. 4-6 illustrate several different print patterns that may be used for applying a binder material to a basesheet in accordance with this invention. As illustrated in FIG. 4, the pattern may comprise a succession of discrete dots. In one embodiment, for instance, the dots can be spaced so that there are approximately from about 25 to about 35 dots per inch (25.4 mm) in the machine direction and/or the cross-machine direction. The dots can have a diameter, for example, of from about 0.01 inch (0.25 mm) to about 0.03 inch (0.76 mm). In one particular embodiment, the dots can have a diameter of about 0.02 inch (0.51 mm) and can be present in the pattern so that approximately 28 dots per inch (25.4 mm) extend in both the machine direction and the cross-machine direction. Besides dots, various other discrete shapes such as elongated ovals or rectangles can also be used when printing the binder material onto the sheet.

FIG. 5 shows a print pattern in which the binder material print pattern is made up of discrete multiple deposits that are each comprised of three elongated hexagons. In one embodiment, each hexagon can be about 0.02 inch (0.51 mm) long and can have a width of about 0.006 inch (0.15 mm). Approximately 35 to 40 deposits per inch (25.4 mm) can be spaced in the machine direction and the cross-machine direction.

FIG. 6 illustrates an alternative binder material pattern in which the binder material is printed onto the sheet in a reticulated pattern. The dimensions are similar to those of the dot pattern of FIG. 4. Reticulated patterns, which provide a continuous network of binder material, may result in relatively greater sheet strength than comparable patterns of discrete elements, such as the dot pattern of FIG. 4. It will be appreciated that many other patterns, in addition to those illustrated above, can also be used depending on the desired properties of the final product.

With reference again to FIG. 3, after the binder material 70 is applied, the sheet 52 is adhered to a heated creping cylinder 75 by a press roll 76. The sheet 52 is carried on the surface of the heated creping cylinder 75 for a distance and then removed therefrom by the action of a creping blade 78. The creping blade 78 performs a controlled pattern creping operation on the side of the sheet 52 to which the binder material 70 was applied.

Once creped, the sheet 52 is pulled through an optional drying station 80. The drying station can include any form of a heating unit, such as an oven energized by infrared heat, microwave energy, hot air, or the like. Alternatively, the drying station may comprise other drying methods such as photo-curing, UV-curing, corona discharge treatment, electron beam curing, curing with reactive gas, curing with heated air such as through-air heating or impingement jet heating, infrared heating, contact heating, inductive heating, microwave or RF heating, and the like. Depending upon the binder material selected, however, drying station 80 may not

be needed. Once passed through the drying station 80, the sheet 52 can be wound into a roll of material or product 85.

In certain instances the binder composition may be selected not only to assist in creping the web but also for improving one or more physical properties of the web such as, for example, dry strength, wet strength, stretch and tear resistance. Particular binder compositions that may be used in the present invention include latex compositions. The latex composition may comprise a non-carboxylated latex emulsion or a carboxyl-functional latex emulsion polymer. Non-carboxylated latex emulsions useful in the present invention may comprise an aqueous polymer dispersion of vinyl acetate and ethylene. Suitable non-carboxylated latex emulsions include vinyl acetate and ethylene emulsions such as Vinnapas<sup>TM</sup> EZ123, commercially available from Wacker Polymers, LP (Allentown, PA). In other instances the binder composition may comprise a carboxyl-functional latex polymers such as Vinnapas<sup>TM</sup> EP1133, commercially available from Wacker Polymers, LP (Allentown, PA).

Latex polymers useful in the present invention may comprise unsaturated monomers, such as vinyl acetate and ethylene monomers, polymerized in the presence of surfactants and initiators to produce emulsion-polymerized polymer particles. Unsaturated monomers contain carbon-to-carbon double bond unsaturation and generally include vinyl monomers, styrenic monomers, acrylic monomers, allylic monomers, acrylamide monomers, as well as carboxyl functional monomers. Vinyl monomers include vinyl esters such as vinyl acetate, vinyl propionate and similar vinyl lower alkyl esters, vinyl halides, vinyl aromatic hydrocarbons such as styrene and substituted styrenes, vinyl aliphatic monomers such as alpha olefins and conjugated dienes, and vinyl alkyl ethers such as methyl vinyl ether and similar vinyl lower alkyl ethers. Acrylic monomers include lower alkyl esters of acrylic or methacrylic acid having an alkyl ester chain from one to twelve carbon atoms as well as aromatic derivatives of acrylic and methacrylic acid. Useful acrylic monomers include, for instance, methyl, ethyl, butyl, and propyl acrylates and methacrylates, 2-ethyl hexyl acrylate and methacrylate, cyclohexyl, decyl, and isodecyl acrylates and methacrylates, and similar various acrylates and methacrylates.

In certain embodiments the latex polymers may comprise a carboxyl-functional latex polymer comprising copolymerized carboxyl-functional monomers such as acrylic and methacrylic acids, fumaric or maleic or similar unsaturated dicarboxylic acids, where the preferred carboxyl monomers are acrylic and methacrylic acid. In certain instances the carboxyl-functional latex polymers may comprise by weight from about 1 to about 50 percent copolymerized carboxyl monomers with the balance being other copolymerized ethylene monomers. Suitable carboxyl-functional latex polymers include carboxylated vinyl acetate-ethylene polymer emulsions such as Vinnapas<sup>TM</sup> EP1133, commercially available from Wacker Polymers, LP (Allentown, PA).

In certain instances the binder composition may optionally contain an anti-blocking additive designed to modify the surface chemistry or characteristics of the binder film on the basesheet. Suitable anti-blocking additives generally do not react chemically with the binder and may include: 1) surfactants, including anionic surfactants such as sodium and potassium salts of stearic, palmitic, oleic, lauric, and tall oil fatty acids, and non-ionic surfactants such as polyoxyethylene glycols reacted to a lyophilic compound; 2) non-reactive additives, such as silicones, waxes, oils, designed to modify the surface chemistry of at least one outer surface of the web to reduce blocking; and 3) soluble or insoluble crystals, such

as sugars, talc, clay, and the like, designed to reside on the surface of the binder film and thus reduce its propensity to cause blocking to an adjacent web surface. The amount of the anti-blocking additive in the binder composition, relative to the amount of carboxyl-functional latex emulsion polymer on a weight percent solids basis, can be from about 1 to about 25 percent, more specifically from about 5 to about 20 percent and more specifically from about 10 to about 15 percent.

Accordingly, in certain embodiments, binders useful in the present invention may consist essentially of a non-crosslinked latex polymer, such as a vinyl acetate-ethylene latex polymer, and optionally an anti-blocking agent, such as a polysaccharide, to prevent blocking upon drying of the tissue web.

In certain preferred embodiments it may be desirable to form the inventive tissue products using a binder that is substantially free from polyfunctional aldehydes, such as glyoxalated polyacrylamide and glyoxal, and azetidinium-functional cross-linking polymers, such as polyamide-epichlorohydrin (PAE) resins and polyamide-polyamine-epichlorohydrin (PPE) resins. Thus, in a preferred embodiment the latex polymer, which may comprise either a non-carboxylated or a carboxylated latex polymer, is not subjected to crosslinking before or after it is applied to the tissue web.

In certain instances the binder composition may be applied to the base web in a preselected pattern. In one embodiment, for instance, the binder composition can be applied to the web in a reticular pattern, such that the pattern is interconnected forming a net-like design or grid on the surface. In other embodiments the binder composition may be applied to the web in a pattern that represents a succession of discrete shapes. For example, the binder composition may be applied in a pattern of discrete dots. Despite consisting of discrete shapes, such patterns provide the desired physical properties without covering a substantial portion of the surface area of the web.

In certain preferred embodiments the binder composition is applied to only one side of the web so as to cover from about 15 to about 75 percent of the surface area of the web. More particularly, in most applications, the binder composition will cover from about 20 to about 60 percent of the surface area of the web. The total amount of binder composition applied to the web can be in the range of from about 1 to about 25 percent by weight, such as from about 2 to about 10 percent by weight, based upon the total weight of the web.

In the embodiment shown in FIG. 3 only one side of the web is treated with a binder composition leaving an untreated side. Leaving one side of the tissue web untreated may provide various benefits and advantages under some circumstances. For instance, the untreated side may increase the ability of the tissue web to absorb liquids faster. Further, the untreated side may have a greater texture than if the side were treated with a binder composition.

Further, the process illustrated in FIG. 3 represents only one possible method for applying a binder composition to the web. Other application methods may be suitable for applying a binder composition to the web. For example, various printing methods can be used to print the binder composition onto the web depending upon the particular application. Such printing methods can include direct gravure printing, offset gravure printing, or flexographic printing.

Generally, the tissue webs and products of the present invention have a binder composition applied to one or more

outer surfaces, as described above, but have not been subjected to additional treatment with a softening composition. As used herein, the term "softening composition" refers to any chemical composition which improves the tactile sensation perceived by the end user who holds a particular tissue product and rubs it across the skin. Softening compositions commonly used in the art include, for example, basic waxes such as paraffin and beeswax and oils such as mineral oil and silicone oil, including polysiloxanes and more particularly amino-functional polysiloxane, as well as petrolatum and more complex lubricants and emollients such as quaternary ammonium compounds with long alkyl chains, functional silicones, fatty acids, fatty alcohols and fatty esters.

In other instances the basesheets prepared as described above may be subjected to embossing and plying to produce the inventive tissue products. For example, the tissue products of the present invention may be provided as multi-ply products comprising two or more plies, such as two, three or four plies, where the plies are embossed and laminated together. In one embodiment, the multi-ply product of the present invention may be produced using an embossing-laminating device, such as those described in U.S. Pat. Nos. 3,556,907, 3,867,225 and 5,339,730, the contents of which are incorporated herein in a manner consistent with the present disclosure. For example, two plies may be embossed separately, each between an embossing roller and a counter-roller or pressure roller. The two plies may then be brought into facing relation with one another and joined so that the protuberances of one ply are nested between the protuberances of the other ply. Typically, lamination of the two plies is obtained between one of the embossing rollers and a laminating roller, while the two embossing rollers do not touch.

In a particularly preferred embodiment, the invention provides a multi-ply tissue product comprising at least first and second embossed and creped tissue plies. The plies may further comprise a non-crosslinked latex polymer disposed on at least one outer surface thereof. The embossed plies may comprise an embossing pattern that provides the product with a visual aesthetic and enhances the bulk of the product, such that the product has a bulk greater than about 8.0 cc/g, such as greater than about 9.0 cc/g and more preferably greater than about 10.0 cc/g.

#### Test Methods

##### Basis Weight

Prior to testing, all samples are conditioned under TAPPI conditions ( $23\pm1^\circ\text{ C.}$  and  $50\pm2$  percent relative humidity) for a minimum of 4 hours. Basis weight of sample is measured by selecting twelve (12) products (also referred to as sheets) of the sample and making two (2) stacks of six (6) sheets. In the event the sample consists of perforated sheets of bath or towel tissue, the perforations must be aligned on the same side when stacking the usable units. A precision cutter is used to cut each stack into exactly  $10.16\times10.16\text{ cm}$  ( $4.0\times4.0$  inch) squares. The two stacks of out squares are combined to make a basis weight pad of twelve (12) squares thick. The basis weight pad is then weighed on a top loading balance with a minimum resolution of 0.01 grams. The top loading balance must be protected from air drafts and other disturbances using a draft shield. Weights are recorded when the readings on the top loading balance become constant. The mass of the sample (grams) per unit area (square meters) is calculated and reported as the basis weight, having units of grams per square meter (gsm).

##### Caliper

Caliper is measured in accordance with TAPPI test methods Test Method T 580 pm-12 "Thickness (caliper) of towel, tissue, napkin and facial products." The micrometer used for carrying out caliper measurements is an Emveco 200-A Tissue Caliper Tester (Emveco, Inc., Newberg, OR). The micrometer has a load of 2 kilopascals, a pressure foot area of 2,500 square millimeters, a pressure foot diameter of 56.42 millimeters, a dwell time of 3 seconds and a lowering rate of 0.8 millimeters per second.

##### Slough

The Slough test provides a quantitative measure of the abrasion resistance of a tissue sample. More specifically, the test measures the resistance of a material to an abrasive action when the material is subjected to a horizontally reciprocating surface abrader. The equipment used to measure Slough is similar to that described in U.S. Pat. No. 6,808,595, the disclosure of which is incorporated by reference herein in a manner consistent with the present invention. The abrading spindle consists of a stainless-steel rod, approximately 1.25 cm (0.495 inches) in diameter and 15.25 cm (6 inches) in length. The abrasive portion of the abrading spindle is 10.8 cm (4.25 inches) in length and consists of 18/22 abrasion coating (commercially available from Superabrasives, Inc., Wixom, MI) applied around the entire circumference of the abrading spindle. The abrading spindle is mounted perpendicularly to the face of the instrument such that the abrasive portion of the abrading spindle extends out its entire distance from the face of the instrument. On each side of the abrading spindle is located a pair of clamps, one movable and one fixed. The clamps are spaced 10 cm (4 inches) apart and centered about the abrading spindle. The movable clamp (weighing approximately 21 grams) is allowed to slide freely in the vertical direction, the weight of the movable clamp providing the means for ensuring a constant tension of the tissue sheet sample over the surface of the abrading spindle. Instruments for measuring Slough according to the present invention are available at Accelerated Analytical Laboratories (Milwaukee, WI).

Prior to testing, any loose dust should be removed from the abrading spindle with compressed air. If other debris is present on the abrading spindle, the spindle may be washed in warm water and dish detergent, rinsed with distilled water and dried in an oven. In the event the abrading spindle is washed prior to use, care must be taken to ensure that all cleaning solution is rinsed from the abrading spindle and that it is completely dry before use.

Samples are conditioned under TAPPI conditions ( $23\pm1^\circ\text{ C.}$  and  $50\pm2$  percent relative humidity) for a minimum of 4 hours prior to testing. For perforated bath tissue products, samples are first prepared by unrolling the tissue and separating into lengths of 3 sheets. Using a precision cutter, such as a JDC-3 cutter (commercially available from Thwing-Albert Instrument Company, Philadelphia, PA), each sample is cut to a size of  $177.8\pm13\text{ mm}$  ( $7.0\pm0.5$  inches) in the machine direction (MD) by  $76.2\pm1\text{ mm}$  ( $3.0\pm0.04$  inches) in the cross-machine direction (CD). When cutting perforated bath tissue products, as illustrated in FIG. 7, the sample 100 is cut such that the sample 100 has a first end 102 having a length of about 25.4 mm (1 inch) and a second end 104 having a length of about 50.8 mm (2 inches) which ensures that the spindle does not abrade over the perforations 105, 107 in the sample 100.

When testing rolled and perforated bath tissue products testing should be done on the outside surface of the roll as it is unwound. Generally rolled and perforated bath tissue

products are not separated into individual plies prior to testing and the outer surface of the product, as it is unwound from the roll, is tested. When testing folded facial tissue products, the product is separated into individual plies and the outward facing side of one of the outer plies is tested.

Each tissue sheet sample is weighed to the nearest 0.1 mg. One end of the tissue sheet sample is clamped to the fixed clamp, the sample is then loosely draped over the abrading spindle and clamped into the sliding clamp. The entire width of the sample should be in contact with the abrading spindle. The sliding clamp is then allowed to fall providing constant tension across the abrading spindle. The entire width of the tissue sheet sample should be in contact with the abrading spindle.

Once the sample is secured the test begins by moving the abrading spindle back and forth at an approximate 15-degree angle from the centered vertical centerline in a reciprocal horizontal motion against the tissue sample for 40 cycles at a speed of  $73.5 \pm 0.5$  cycles per minute. As the spindle cycles, it is also rotated counterclockwise (when looking at the front of the instrument) at an approximate speed of 5 RPMs. Once the 40 cycles are complete, the tissue sample is removed from the jaws with the fingertips and both sides of the sample are blown with air having a flow rate of approximately 3.4 scfm for approximately 13 seconds to remove debris.

The tissue sheet sample is then weighed to the nearest 0.1 mg and the weight loss calculated. The difference between the initial weight and the weight after testing is the amount of Slough. Ten samples are tested and the average weight loss value in milligrams (mg) is recorded, which is the Slough value for the sample.

#### Burst Strength (Wet or Dry)

Burst Strength is measured using an EJA Burst Tester (series #50360, commercially available from Thwing-Albert Instrument Company, Philadelphia, PA). The test procedure is according to TAPPI T570 pm-00 except the test speed. The test specimen is clamped between two concentric rings whose inner diameter defines the circular area under test. A penetration assembly, the top of which is a smooth, spherical steel ball, is arranged perpendicular to and centered under the rings holding the test specimen. The penetration assembly is raised at 6 inches per minute such that the steel ball contacts and eventually penetrates the test specimen to the point of specimen rupture. The maximum force applied by the penetration assembly at the instant of specimen rupture is reported as the burst strength in grams force (gf) of the specimen.

The penetration assembly consists of a spherical penetration member which is a stainless steel ball with a diameter of  $0.625 \pm 0.002$  inches ( $15.88 \pm 0.05$  mm) finished spherical to 0.00004 inches (0.001 mm). The spherical penetration member is permanently affixed to the end of a  $0.375 \pm 0.01$  inch ( $9.525 \pm 0.254$  mm) solid steel rod. A 2000 gram load cell is used and 50 percent of the load range, i.e., 0-1000 g is selected. The distance of travel of the probe is such that the upper most surface of the spherical ball reaches a distance of 1.375 inches (34.9 mm) above the plane of the sample clamped in the test. A means to secure the test specimen for testing consisting of upper and lower concentric rings of approximately 0.25 inches (6.4 mm) thick aluminum between which the sample is firmly held by pneumatic clamps operated under a filtered air source at 60 psi. The clamping rings are  $3.50 \pm 0.01$  inches ( $88.9 \pm 0.3$  mm) in internal diameter and approximately 6.5 inches (165 mm) in outside diameter. The clamping surfaces of the clamping rings are coated with a commercial grade of neoprene

approximately 0.0625 inches (1.6 mm) thick having a Shore hardness of 70-85 (A scale). The neoprene needs not cover the entire surface of the clamping ring but is coincident with the inner diameter, thus having an inner diameter of  $3.50 \pm 0.01$  inches ( $88.9 \pm 0.3$  mm) and is 0.5 inches (12.7 mm) wide, thus having an external diameter of  $4.5 \pm 0.01$  inches ( $114 \pm 0.3$  mm). For each test a total of 3 sheets of product are combined.

The sheets are stacked on top of one another in a manner such that the machine direction of the sheets is aligned. Where samples comprise multiple plies, the plies are not separated for testing. In each instance the test sample comprises 3 sheets of product. For example, if the product is a 2-ply tissue product, 3 sheets of product totaling 6 plies are tested. If the product is a single ply tissue product, then 3 sheets of product totaling 3 plies are tested.

Samples are conditioned under TAPPI conditions for a minimum of four hours and cut into  $127 \times 127 \pm 5$  mm squares. For wet burst measurement, after conditioning the samples were wetted for testing with 0.5 mL of deionized water dispensed with an automated pipette. The wet sample is tested immediately after insulating.

The peak load (gf) and energy to peak (g-cm) are recorded and the process repeated for all remaining specimens. A minimum of five specimens are tested per sample and the peak load average of five tests is reported.

#### Tensile

Tensile testing is conducted on a tensile testing machine maintaining a constant rate of elongation and the width of each specimen tested is 3 inches. Testing is conducted under TAPPI conditions. Prior to testing samples are conditioned under TAPPI conditions ( $23 \pm 1^\circ$  C. and  $50 \pm 2$  percent relative humidity) for at least 4 hours and then cutting a  $3 \pm 0.05$  inches ( $76.2 \pm 1.3$  mm) wide strip in either the machine direction (MD) or cross-machine direction (CD) orientation using a JDC Precision Sample Cutter (Thwing-Albert Instrument Company, Philadelphia, PA, Model No. JDC 3-10, Serial No. 37333) or equivalent. The instrument used for measuring tensile strengths was an MTS Systems Sintech 11S, Serial No. 6233. The data acquisition software was MTS TestWorks® for Windows Ver. 3.10 (MTS Systems Corp., Research Triangle Park, NC). The load cell was selected from either a 50 Newton or 100 Newton maximum, depending on the strength of the sample being tested, such that the majority of peak load values fall between 10 to 90 percent of the load cell's full-scale value. The gauge length between jaws was  $4 \pm 0.04$  inches ( $101.6 \pm 1$  mm) for facial tissue and towels and  $2 \pm 0.02$  inches ( $50.8 \pm 0.5$  mm) for bath tissue. The crosshead speed was  $10 \pm 0.4$  inches/min ( $254 \pm 1$  mm/min), and the break sensitivity was set at 65 percent. The sample was placed in the jaws of the instrument, centered both vertically and horizontally. The test was then started and ended when the specimen broke. The peak load was recorded as either the "MD tensile strength" or the "CD tensile strength" of the specimen depending on direction of the sample being tested. Ten representative specimens were tested for each product or sheet and the arithmetic average of all individual specimen tests was recorded as the appropriate MD or CD tensile strength having units of grams per three inches ( $g/3"$ ). Tensile energy absorbed (TEA) and slope are also calculated by the tensile tester. TEA is reported in units of  $g \cdot cm/cm^2$  and slope is recorded in units of kilograms (kg). Both TEA and Slope are directionally dependent and thus MD and CD directions are measured independently.

All products were tested in their product forms without separating into individual plies. For example, a 2-ply prod-

uct was tested as two plies and recorded as such. In the tensile properties of basesheets were measured, the number of plies used varied depending on the intended end use. For example, if the basesheet was intended to be used for 2-ply product, two plies of basesheet were combined and tested. Surface Smoothness

Surface smoothness was measured using an EMTEC Tissue Softness Analyzer ("TSA") (Emtec Electronic GmbH, Leipzig, Germany). The TSA comprises a rotor with vertical blades which rotate on the tissue sample applying a defined contact pressure. The blades are pressed against the sample with a load of 100 mN and the rotational speed of the blades is two revolutions per second. Contact between the vertical blades and the tissue sample creates vibrations, which are sensed by a vibration sensor. The sensor transmits a signal to a PC for processing and display. The signal is displayed as a frequency spectrum. The frequency spectrum is analyzed by the associated TSA software to determine the amplitude of the frequency peak occurring in the range between 200 to 1000 Hz. This peak is generally referred to as the TS750 value (having units of dB V<sup>2</sup> rms) and represents the surface smoothness of the tissue sample. A high amplitude peak correlates to a rougher surface, while a low amplitude peak correlates to a smoother surface.

Tissue product samples were prepared by cutting a circular sample having a diameter of 112.8 mm. All samples were allowed to equilibrate at TAPPI conditions for at least 24 hours prior to completing the TSA testing. After conditioning, each sample was tested as-is, i.e., multi-ply products were tested without separating the sample into individual plies. The sample is secured, and the measurements are started via the PC. The PC records, processes and stores all of the data according to standard TSA protocol. The reported TS750 value is the average of five replicates, each one with a new sample.

## EXAMPLES

Basesheets were made using a through-air dried paper-making process commonly referred to as "uncreped through-air dried" ("UCTAD") and generally described in U.S. Pat. No. 5,607,551, the contents of which are incorporated herein in a manner consistent with the present disclosure. Basesheets with a target bone dry basis weight of about 25 gsm were produced. The basesheets were then print creped and converted into multi-ply tissue products by plying, embossing, and winding about a core. Neither the basesheets nor the resulting multi-ply tissue product were subjected to surface treatment with silicones, waxes, lotions or quaternary ammonium compounds comprising alkyl chains.

Basesheets were prepared using a three-layered headbox to form a web having a first outer layer, also referred to as the fabric or fabric contacting layer, a middle layer, and a second outer layer, also referred to as the air contacting or air layer. The furnish split, which consisted of eucalyptus hardwood kraft pulp (EHWK) and northern softwood kraft pulp (NSWK), and treatment of the various furnish layers is detailed in Table 2, below.

TABLE 2

| Layer  | Fiber Type | Fiber Wt % | Chemical Add-On (kg/MT) |
|--------|------------|------------|-------------------------|
| Fabric | EHWK       | 30         | ProSoft™ TQ-1003 (1.5)  |
| Middle | NSWK       | 40         | Fennobond™ 3300 (0.5)   |
| Air    | EHWK       | 30         | —                       |

Each furnish was diluted to approximately 0.2 percent consistency and delivered to a layered headbox and depos-

ited on a Voith Fabrics TissueForm V forming fabric (commercially available from Voith Fabrics, Appleton, WI). The wet web was vacuum dewatered to approximately 25 percent consistency and then subjected to rush transfer when transferred to the transfer fabric. The transfer fabric was the fabric described as "Fred" in U.S. Pat. No. 7,611,607 (commercially available from Voith Fabrics, Appleton, WI). The rush transfer rate was 28 percent. The web was then transferred to a Tissue Max EX through-air drying fabric (commercially available from Voith Fabrics, Appleton, WI). The web was dried with a through-air-dryer resulting in dried tissue web. The single ply basesheet physical properties are summarized in Table 3, below.

TABLE 3

|             | BW<br>(gsm) | GMT<br>(g/3") | MD<br>Slope<br>(kg) | MD<br>TEA<br>cm/<br>cm <sup>2</sup> | CD<br>Tensile<br>(g/3") | CD<br>Slope<br>(kg) | CD<br>TEA<br>cm/<br>cm <sup>2</sup> | Wet<br>CD<br>Tensile<br>(g/3") |
|-------------|-------------|---------------|---------------------|-------------------------------------|-------------------------|---------------------|-------------------------------------|--------------------------------|
|             |             |               |                     |                                     |                         |                     |                                     |                                |
| Inventive 1 | 25.0        | 1389          | 11.1                | 28.1                                | 1104                    | 15.1                | 8.15                                | 136                            |
| Inventive 2 | 25.3        | 1418          | 13.1                | 29.1                                | 1111                    | 14.7                | 7.70                                | 140                            |
| Inventive 3 | 25.0        | 1353          | 12.1                | 28.3                                | 1052                    | 15.0                | 7.90                                | 149                            |
| Inventive 4 | 25.1        | 1403          | 13.1                | 29.1                                | 1094                    | 16.4                | 7.85                                | 139                            |
| Inventive 5 | 24.5        | 1325          | 11.2                | 26.3                                | 1033                    | 16.9                | 7.10                                | 120                            |

The dried tissue web was fed to a gravure printing line, similar to that shown in FIG. 3, traveling at about 1,000 feet per minute where a latex polymer was printed onto the surface of the sheet. The binder composition was varied for each of the sample codes as indicated in Table 4, below. Each of the binders are commercially available from Wacker Polymers, LP (Allentown, PA).

TABLE 4

| 40 | Sample      | Binder           | Binder<br>Compo-<br>sition<br>Solids (%) | Binder<br>Compo-<br>sition<br>(cps) | Binder<br>Compo-<br>sition<br>pH |
|----|-------------|------------------|------------------------------------------|-------------------------------------|----------------------------------|
|    | Inventive 1 | Vinnapas™ 315    | 30                                       | 36                                  | 6.06                             |
|    | Inventive 2 | Vinnapas™ 400    | 30                                       | 37                                  | 6.00                             |
|    | Inventive 3 | Vinnapas™ 4600   | 30                                       | 25                                  | 6.88                             |
| 45 | Inventive 4 | Vinnapas™ EP1133 | 15                                       | 17                                  | 6.16                             |
|    | Inventive 5 | Vinnapas™ EZ123  | 30                                       | 34                                  | 5.92                             |

The binder composition was prepared by mixing the binder with water and a nonionic surfactant (Advantage™ 1529, commercially available from Solenis, Wilmington, DE). The pH of the latex-based binder composition was adjusted using NaOH to a pH of approximately 6.0 and allowed to mix for approximately 5-30 minutes prior to use in the gravure printing operation. The viscosity of the latex-based binder composition was measured at room temperature using a Brookfield™ Synchro-lectric Model RVT (Brookfield Engineering Laboratories Inc., Stoughton, MA) viscometer with a #1 spindle operating at 20 rpm.

The first side of the dried web was printed with a binding composition using direct rotogravure printing in a pattern as shown in FIG. 5. The pattern comprises three elongated hexagons having a length of about 0.02 inch (0.51 mm) and a width of about 0.006 inch (0.15 mm). After printing, the sheet was pressed against and doctored off a rotating drum, which had a surface temperature of approximately 126° C.

The print creped tissue web was subjected to further converting to produce a two-ply tissue product. Individual plies were plied together and embossed using an embossing-

laminating device, such as the device described in U.S. Pat. No. 3,867,225. The individual plies were arranged such that the surface printed with the binder composition formed the two outer surfaces of the two-ply tissue product.

The two-ply tissue product was converted into a finished rolled tissue product by winding the multi-ply and embossed tissue product about a core. Finished products were subject to physical testing, the results of which are summarized in Tables 5 and 6, below.

TABLE 5

| Sample      | Basis Weight (gsm) | Caliper (μm) | Bulk (cc/g) | GMT (g/3") | GM Slope (kg) | GM TEA (gf · cm/cm <sup>2</sup> ) | GM Stretch (%) | CD Dry Tensile (g/3") | CD Wet Tensile (g/3") |
|-------------|--------------------|--------------|-------------|------------|---------------|-----------------------------------|----------------|-----------------------|-----------------------|
| Inventive 1 | 57.6               | 516          | 9.0         | 1977       | 10.00         | 30.2                              | 21.5           | 1568                  | 163                   |
| Inventive 2 | 56.8               | 538          | 9.5         | 1365       | 5.70          | 23.1                              | 23.9           | 1076                  | 137                   |
| Inventive 3 | 57.1               | 490          | 8.6         | 1805       | 8.12          | 28.6                              | 23.1           | 1349                  | 173                   |
| Inventive 4 | 55.2               | 450          | 8.1         | 1616       | 7.26          | 24.1                              | 21.5           | 1221                  | 155                   |
| Inventive 5 | 55.7               | 511          | 9.2         | 2490       | 8.59          | 42.3                              | 26.5           | 1696                  | 251                   |

TABLE 6

| Sample      | Stiffness Index | TEA Index | Wet/Dry Ratio | Tensile Ratio |
|-------------|-----------------|-----------|---------------|---------------|
| Inventive 1 | 5.06            | 1.53      | 0.104         | 1.59          |
| Inventive 2 | 4.17            | 1.69      | 0.127         | 1.61          |
| Inventive 3 | 4.50            | 1.58      | 0.128         | 1.79          |
| Inventive 4 | 4.49            | 1.49      | 0.127         | 1.75          |
| Inventive 5 | 3.45            | 1.70      | 0.148         | 2.15          |

Additional inventive samples were prepared by preparing basesheets substantially as described in the example above. The basesheets had a target bone dry basis weight of about 22 gsm. Basesheets were prepared using a three-layered headbox to form a web having a first outer layer and a second outer layers and a middle layer disposed there between. The basesheet comprised 60 wt % EHWK, which was used to form the two outer layers, and 40 wt % NSWK, which formed the middle layer. Strength of the basesheet was controlled by refining the NSWK or by the addition of Fennobond™ 3300 to the middle layer furnish. The basesheets converted by print creping, calendering, embossing, plying and winding about a core as described above. Finished products were subject to physical testing, the results of which are summarized in Tables 7 and 8, below.

TABLE 7

| Sample      | Basis Weight (gsm) | Caliper (μm) | GMT (g/3") | GM Slope (kg) | GM TEA (gf · cm/cm <sup>2</sup> ) | CD Dry Tensile (g/3") | CD Wet Tensile (g/3") |
|-------------|--------------------|--------------|------------|---------------|-----------------------------------|-----------------------|-----------------------|
| Inventive 6 | 48.6               | 541          | 956        | 4.90          | 14.54                             | 775                   | 125                   |
| Inventive 7 | 48.6               | 577          | 1114       | 5.75          | 16.58                             | 835                   | 139                   |

TABLE 8

| Sample      | Stiffness Index | TEA Index | Wet/Dry Ratio | Slough (mg) | Slosh (sec.) | TS750 |
|-------------|-----------------|-----------|---------------|-------------|--------------|-------|
| Inventive 6 | 5.06            | 1.52      | 0.161         | 0.44        | 34           | 25.6  |
| Inventive 7 | 4.17            | 1.48      | 0.166         | 0.96        | 50           | 28.1  |

## 22

### Embodiments

First embodiment: A non-treated and creped multi-ply tissue product comprising a first non-treated and creped tissue ply and a second non-treated and creped tissue ply, the non-treated and creped multi-ply tissue product having a geometric mean tensile (GMT) from about 1,000 to about 2,500 g/3" and a geometric mean tensile energy absorption (GM TEA) greater than about 20 gf·cm/cm<sup>2</sup>.

Second embodiment: The product of the first embodiment wherein a non-crosslinked vinyl acetate-ethylene polymer is disposed on an outer surface of the first or second tissue ply.

Third embodiment: The product of any one of embodiments 1 or 2 wherein a non-crosslinked vinyl acetate-ethylene polymer and at least one anti-blocking agent selected from the group consisting of polysaccharides and surfactants is disposed on an outer surface of the first or second tissue ply.

Fourth embodiment: The product of any one of embodiments 1 through 3 wherein the first and second plies are print creped and comprise a non-crosslinked vinyl acetate-ethylene polymer disposed on at least one outer surface.

Fifth embodiment: The product of any one of embodiments 1 through 4 wherein the product does not comprise a permanent wet strength agent.

Sixth embodiment: The product of any one of embodiments 1 through 5 having a TS750 value less than 40.0.

Seventh embodiment: The product of any one of embodiments 1 through 6 having a dry burst strength greater than about 700 gf, such as from about 700 to about 1,000 gf.

Eighth embodiment: The product of any one of embodiments 1 through 7 having a Slough less than about 5.0 mg.

Ninth embodiment: The product of any one of embodiments 1 through 8 having a Stiffness Index from about 5.0 to about 10.0.

Tenth embodiment: The product of any one of embodiments 1 through 9 having a TEA Index greater than about 1.50.

Eleventh embodiment: The product of any one of embodiments 1 through 10 having a geometric mean stretch (GM Stretch) greater than about 20 percent.

Twelfth embodiment: The product of any one of embodiments 1 through 11 having a GMT from about 1,500 to about 2,200 g/3".

Thirteenth embodiment: The product of any one of embodiments 1 through 12 having a GM TEA from about 25 to about 45 gf·cm/cm<sup>2</sup>.

Fourteenth embodiment: The product of any one of embodiments 1 through 13 having a Wet/Dry Ratio greater than about 0.130.

Fifteenth embodiment: The product of any one of embodiments 1 through 14 having a wet CD tensile strength greater than about 120 g/3".

Sixteenth embodiment: The product of any one of embodiments 1 through 15 wherein each ply comprises two or more layers, wherein at least one layer comprises soft-wood fibers and at least one layer comprises hardwood fibers, and each ply has an outer surface having a non-crosslinked vinyl acetate-ethylene polymer disposed thereon. In certain instances, the non-crosslinked vinyl acetate-ethylene polymer is disposed on the outer surface in a pattern such as, for example, a continuous network.

Seventeenth embodiment: The product of any one of embodiments 1 through 16 having a Slosh time less than 2 minutes.

What is claimed is:

1. A non-treated and creped multi-ply tissue product comprising:
    - a. a first creped, non-treated, through-air dried tissue ply;
    - b. a second creped, non-treated, through-air dried tissue ply;
    - c. a creping composition disposed on the first and the second tissue plies; and
    - d. a plurality of embossments disposed on the first tissue ply or the second tissue ply,

wherein the product is devoid of a permanent wet strength agent and has a geometric mean tensile strength (GMT) from about 1,000 to about 2,500 g/3", a Wet/Dry Ratio from about 0.100 to about 0.200 and a geometric mean tensile energy absorption (GM TEA) from about 20 gf-cm/cm<sup>2</sup> to about 40 gf-cm/cm<sup>2</sup>.
  2. The tissue product of claim 1 having a GMT from about 1,000 to about 2,200 g/3".
  3. The tissue product of claim 1 having a GMT from about 1,500 to about 2,200 g/3".
  4. The tissue product of claim 1 having a Stiffness Index from about 2.5 to about 5.0.
- 10
5. The tissue product of claim 1 having a geometric mean slope (GM Slope) about 5.0 to about 10.0 kg.
  6. The tissue product of claim 1 having a GM Slope from about 5.0 to about 8.0 kg.
  7. The tissue product of claim 1 having a GM TEA from about 25 to about 45 gf-cm/cm<sup>2</sup>.
  8. The tissue product of claim 1 having a TEA Index from about 1.50 to about 2.25.
  9. The tissue product of claim 1 having a Slosh Time less than about 2 minutes.
  10. The tissue product of claim 1 having a basis weight from about 48.0 to about 60.0 gsm.
  11. The tissue product of claim 1 having a Wet/Dry Ratio from about 0.100 to about 0.175.
  12. The tissue product of claim 1 having a wet CD tensile strength from about 120 to about 200 g/3" and a Wet/Dry Ratio from about 0.100 to about 0.175.
  13. The tissue product of claim 1 having a Slough less than about 5.0 mg.
  14. The tissue product of claim 1 having a dry burst strength greater than about 700 gf.
  15. The tissue product of claim 1 having a geometric mean stretch (GM Stretch) greater than about 20 percent.
  16. The tissue product of claim 1 wherein the creping composition comprises a carboxyl-functional latex polymer.
  17. The tissue product of claim 1 wherein the creping composition comprises a non-crosslinked vinyl acetate-ethylene polymer.
  18. The tissue product of claim 1 wherein the first ply or the second ply comprises a temporary wet strength agent.
  19. The tissue product of claim 18 wherein the temporary wet strength agent comprises a glyoxalated polyacrylamide polymer.
- 15
- 20
- 25
- 30

5. The tissue product of claim 1 having a geometric mean slope (GM Slope) about 5.0 to about 10.0 kg.

6. The tissue product of claim 1 having a GM Slope from about 5.0 to about 8.0 kg.

7. The tissue product of claim 1 having a GM TEA from about 25 to about 45 gf-cm/cm<sup>2</sup>.

8. The tissue product of claim 1 having a TEA Index from about 1.50 to about 2.25.

9. The tissue product of claim 1 having a Slosh Time less than about 2 minutes.

10. The tissue product of claim 1 having a basis weight from about 48.0 to about 60.0 gsm.

11. The tissue product of claim 1 having a Wet/Dry Ratio from about 0.100 to about 0.175.

12. The tissue product of claim 1 having a wet CD tensile strength from about 120 to about 200 g/3" and a Wet/Dry Ratio from about 0.100 to about 0.175.

13. The tissue product of claim 1 having a Slough less than about 5.0 mg.

14. The tissue product of claim 1 having a dry burst strength greater than about 700 gf.

15. The tissue product of claim 1 having a geometric mean stretch (GM Stretch) greater than about 20 percent.

16. The tissue product of claim 1 wherein the creping composition comprises a carboxyl-functional latex polymer.

17. The tissue product of claim 1 wherein the creping composition comprises a non-crosslinked vinyl acetate-ethylene polymer.

18. The tissue product of claim 1 wherein the first ply or the second ply comprises a temporary wet strength agent.

19. The tissue product of claim 18 wherein the temporary wet strength agent comprises a glyoxalated polyacrylamide polymer.

\* \* \* \* \*